

## UNITED STATES PATENT OFFICE

1,938,623

## SPINNING OF ARTIFICIAL FILAMENTS

Camille Dreyfus, New York, N. Y., and William Whitehead, Cumberland, Md., assignors to Celanese Corporation of America, a corporation of Delaware

No Drawing. Application November 20, 1929  
Serial No. 408,667

14 Claims. (Cl. 18—54)

This invention relates to the making of filaments such as yarns, bristles, artificial straw and the like containing organic derivatives of cellulose and which have improved properties.

5 An object of our invention is to produce yarns, filaments and the like containing organic derivatives of cellulose which may be readily delustered. A further object is to prepare yarns containing filaments of very fine denier. An-  
10 other object of our invention is to prepare yarns and fabrics containing organic derivatives of cellulose which have a relatively low scorching point and a relatively high melting point, whereby when the material is ironed at high tem-  
15 perature, it scorches before it melts.

It is very desirable for many purposes to pro-  
duce yarns of organic derivatives of cellulose  
that may be readily delustered. Also it is de-  
sirable to prepare yarns which contain filaments  
20 of very low denier. Moreover since textile ma-  
terials containing organic derivatives of cellulose  
tend to melt and stick to the iron when ironed  
with an iron that is at too high a temperature  
it is advantageous that a warning, such as  
25 scorching, be given the operator of the danger  
of the high temperatures. We have found that  
these results may be obtained by employing as  
a spinning dope from which filaments or yarns  
30 are formed, a solution of a derivative of cellulose  
that contains a soap or a compound of a fatty  
acid.

In accordance with our invention we prepare  
filaments containing organic derivatives of cel-  
lulose by extruding a solution of the same in a  
35 suitable solvent and which solution contains a  
soap or a salt of a higher fatty acid through  
orifices of suitable size and shape into an evap-  
orative atmosphere as in dry spinning, or into a  
precipitating bath as in wet spinning.

40 Filaments of any desired size or shape may be  
made in accordance with this invention. While  
we prefer to make fine filaments which are as-  
sociated together to form yarn, heavier filaments  
45 to be employed as artificial bristles or horse hair  
or as artificial straw may be made. Any suit-  
able organic derivatives of cellulose such as or-  
ganic esters of cellulose or cellulose ethers may  
be employed. Examples of organic esters of cel-  
50 lulose are cellulose acetate, cellulose formate,  
cellulose propionate and cellulose butyrate while  
examples of cellulose ethers are ethyl cellulose,  
methyl cellulose and benzyl cellulose.

The solution is formed by dissolving the or-  
ganic derivatives of cellulose in a suitable sol-  
55 vent or solvent mixture. For dry spinning, vol-

atile solvents are employed examples of which  
are acetone, methyl acetate, mixtures of acetone  
and methyl or ethyl alcohol, mixtures of methyl-  
ene chloride and ethyl or methyl alcohol and  
mixtures of ethylene dichloride and ethyl or 60  
methyl alcohol. For wet spinning either a vola-  
tile solvent or a non volatile solvent may be  
employed.

As stated the solution of the derivative of cel-  
lulose contains soap or salt of a higher fatty 65  
acid. Examples of these are potassium ricin-  
oleate, potassium stearate, potassium oleate, so-  
dium ricinoleate, sodium stearate, sodium oleate  
or salts of triethanol amine and fatty acids such  
as triethanol amine stearate, or triethanol amine 70  
oleate. While the amounts of the soap employed  
may vary greatly, we have generally found that  
amounts equal to 1.5 to 10% of the weight of  
the organic derivative of cellulose present in the  
solution produces very satisfactory results. 75

If the dry spinning method is employed, the  
solution or spinning dope is extruded through  
orifices into heated air, nitrogen, carbon di-  
oxide or any other suitable gas. For wet spin-  
ning the dope is extruded into a bath that 80  
causes the precipitation of the derivative of  
cellulose from such solution. In the latter case,  
where the spinning dope comprises solutions of  
cellulose acetate in acetone, an essential constit-  
uent of the precipitating bath is water. 85

The filaments or yarns formed in accordance  
with our invention or fabrics made from such  
yarn are either of subdued lustre or may be  
readily delustered by the action of water or  
other aqueous baths, such as are employed in 90  
scouring and dyeing at comparatively low tem-  
peratures. Moreover if a delustered fabric con-  
structed of yarn made in accordance with this  
invention becomes relustered when ironed while  
damp, the relustering effect that is produced in 95  
spots or on the whole fabric may be destroyed  
by treating the fabric in warm water, where-  
upon the fabric becomes uniformly delustered,  
a result not attained heretofore. The behavior  
of the yarn made in accordance with this in-  
vention with respect to delustering is of par-  
ticular importance in the making of hosiery or  
other knit fabric where a subdued lustre is  
required. 100

Yarn made in accordance with this invention  
is pliable and therefore may be knitted into a  
more closely knitted fabric containing more  
stitches per unit length than is possible with  
yarn made from solutions not containing the  
soaps. 110

Yarn made in accordance with this invention or fabric containing such yarn scorches at temperatures lower than yarn not containing the soaps. Furthermore such fabric has a higher melting point than prior fabric, and has a safe ironing point of 20° C. or more higher than fabric made of yarn not containing the soaps.

Another advantage of this invention is the fact that when certain soaps such as potassium ricinoleate are employed, filaments of 10% or more finer size or denier may be produced.

In order to further illustrate our invention but without being limited thereto, the following specific examples are given.

15

*Example I*

A spinning solution is made by dissolving an acetone soluble cellulose acetate in the following proportions:

|                       | Parts by weight. |
|-----------------------|------------------|
| Cellulose acetate     | 25               |
| Acetone               | 73               |
| Potassium ricinoleate | 2                |

20 The charge is mixed to a homogeneous clear solution, filtered and then extruded through orifices into an evaporative atmosphere. The filaments thus formed are associated together by twisting to form yarn and are wound up on a suitable package.

25 Filaments of much finer denier than heretofore possible may be made. The yarn so formed has the following new and useful properties. Although lustrous when formed, it becomes delustered when submerged even in cold water for a period of time such as 24 hours. It delusters very rapidly when treated in dye or scouring baths at the temperatures ordinarily employed such as 65° C. The fabric containing the yarn so delustered, when ironed damp at elevated temperatures relusters much as has heretofore been the case with prior fabrics made of cellulose acetate. However, in the case of yarns made in the manner herein described, such relustered fabrics become delustered again by simply immersing in warm water. Of course the higher the temperature of the water, the more speedily the relustered fabric becomes delustered. Thus, for example, 15 minute treatment is ample in the case when water of 65° C. is employed, but when water at ordinary temperatures is used several hours treatment is necessary. Fabrics made in accordance with this example which have become relustered in patches by damp ironing, when treated as described, deluster again in the relustered patches and the fabrics show no unevenness of appearance after drying out and ironing while the fabrics are substantially dry.

60

*Example II*

The process of Example I is repeated with the exception that the trioleate of triethanol amine is substituted for the potassium ricinoleate, the yarns having similar properties to those described in Example I are derived.

65 It is to be understood that the foregoing detailed description is given merely by way of illustration and that many variations may be made therein without departing from the spirit of this invention.

Having described our invention what we claim and desire to secure by Letters Patent is:

70 1. Method of making filaments capable of receiving a low lustre comprising extruding a solution containing an organic derivative of cellulose

and a water-soluble salt of a higher fatty acid which is soluble in the organic derivative of cellulose solvent through orifices into a setting fluid which does not alter the solubility of the salt, so that on solidification of the filaments at least some of the water-soluble salt is retained as such in the filaments.

75 2. Method of making filaments capable of receiving a low lustre comprising extruding a solution containing cellulose acetate and a water-soluble salt of a higher fatty acid which is soluble in the cellulose acetate solvent through orifices into a setting fluid which does not alter the solubility of the salt, so that on solidification of the filaments at least some of the water-soluble salt is retained as such in the filaments.

80 3. Method of making filaments capable of receiving a low lustre comprising extruding a solution containing an organic derivative of cellulose and a water-soluble salt of a higher fatty acid which is soluble in the organic derivative of cellulose solvent through orifices into a drying evaporative atmosphere so that on solidification of the filaments at least some of the water-soluble salt is retained as such in the filaments.

85 4. Method of making filaments capable of receiving a low lustre comprising extruding a solution containing cellulose acetate and a water-soluble salt of a higher fatty acid which is soluble in the cellulose acetate solvent through orifices into a drying evaporative atmosphere so that on solidification of the filaments at least some of the water-soluble salt is retained as such in the filaments.

90 5. Method of making filaments capable of receiving a low lustre comprising extruding a solution containing cellulose acetate and an alkali metal ricinoleate through orifices into a drying evaporative atmosphere so that on solidification of the filaments at least some of the alkali metal ricinoleate is retained as such in the filaments.

95 6. Method of making filaments capable of receiving a low lustre comprising extruding a solution containing cellulose acetate and potassium ricinoleate through orifices into a drying evaporative atmosphere so that on solidification of the filaments at least some of the potassium ricinoleate is retained as such in the filaments.

100 7. Method of making filaments capable of receiving a low lustre comprising extruding a solution containing cellulose acetate and a salt of triethanolamine with a fatty acid which is soluble in the cellulose acetate solvent through orifices into a drying evaporative atmosphere so that on solidification of the filaments at least some of the salt is retained as such in the filaments.

105 8. Method of making filaments capable of receiving a low lustre comprising extruding a solution containing cellulose acetate and the trioleate of triethanol amine through orifices into a drying evaporative atmosphere so that on solidification of the filaments at least some of the trioleate of triethanol amine is retained as such in the filaments.

110 9. Filaments or yarns capable of receiving a low lustre, said filaments containing an organic derivative of cellulose and a water-soluble salt of a higher fatty acid.

115 10. Filaments or yarns capable of receiving a low lustre, said filaments containing cellulose acetate and a water-soluble salt of a higher fatty acid.

120 11. Filaments or yarns capable of receiving a low lustre comprising extruding a solution containing cellulose acetate and a water-soluble salt of a higher fatty acid.

a low lustre, said filaments containing cellulose acetate and an alkali metal ricinoleate.

12. Filaments or yarns capable of receiving a low lustre, said filaments containing cellulose acetate and potassium ricinoleate.

13. Filaments or yarns capable of receiving a low lustre, said filaments containing cellulose

acetate and a salt of triethanol amine with a fatty acid.

14. Filaments or yarns capable of receiving a low lustre, said filaments containing cellulose acetate and the trioleate of triethanol amine. 80

CAMILLE DREYFUS.  
WILLIAM WHITEHEAD.

10 85

15 90

20 95

25 100

30 105

35 110

40 115

45 120

50 125

55 130

60 135

65 140

70 145

75 150